

## UNITED STATES PATENT OFFICE

1,944,175

PROCESS OF ODORIZING LIQUEFIED  
PETROLEUM GASESFrederick E. Frey, Bartlesville, Okla., assignor to  
Phillips Petroleum Company, Bartlesville,  
Okla., a corporation of DelawareNo Drawing. Application October 7, 1929  
Serial No. 398,109

3 Claims. (Cl. 44—8)

This invention pertains to the odorizing of liquefied petroleum gas.

It is well known that liquefied petroleum gas such as butane and propane, when mixed with air, form explosive mixtures. As the odor of such petroleum gases is too weak to warn those present where such gases are escaping, the use of liquefied petroleum gas, as a fuel, especially is attended by some danger of fire and explosion from leaks and open jets.

I have discovered that an adequate odor may be imparted to such gases by adding to the same while stored in liquid condition, in a cylinder or the like, an odorous material in sufficient amount to odorize a mixture of the gas with the maximum amount of air that will permit combustion. This may be accomplished by introducing into the cylinder containing the liquefied gas, an odorous material of sufficient volatility to deliver the necessary concentration to the gas, under the high pressure developed in the cylinder. However, very few substances may be employed for this purpose, due to the fact that the gas when utilized, changes from liquid to gaseous condition, and consequently, the proportion of the odorous substance may vary in the gaseous fluid as the content of the cylinder diminishes, as the liquefied gas is used from the same.

In the case of a gas consisting mainly of propane, I have found it advisable to use an odorous material of high volatility, but the number of substances possessing both the required odor strength and volatility is limited. Consequently, special measures must be used to make materials of other than the correct volatility serve the purpose.

Furthermore, it is desirable that the concentration of odor delivered be fairly constant, whether the cylinder is full of liquid fuel or nearly empty.

In accordance with my invention, I have discovered that if propylene is used as an odorizer of propane for example, since it is highly miscible with propane and equally volatile, it will be delivered in fairly constant concentration as the content of the cylinder diminishes.

Therefore, as a part of the present invention, I propose a liquefied fuel consisting essentially of propane and propylene, in which the propylene is present in sufficient quantity to impart an odor to all flammable mixtures with air.

I have also discovered that in odorizing liquefied petroleum or the like, it is not absolutely necessary to use an odorizing substance having

equal volatility to the liquefied gas. For example, if a soluble compound boiling at a temperature somewhat higher than propane, such as dimethylsulfide be used as an odorizer, the concentration delivered will be less than the concentration in the liquid fuel at all times. Consequently, the emptying of a cylinder by evaporation, will cause a continuous increase in the concentration of the odorizer in the liquid, and in the gas delivered. However, I recommend that a soluble liquid of comparatively low vapor pressure, such as kerosene be present in the cylinder containing the mixture of propane and dimethylsulfide, to limit the increase in concentration that can take place when the cylinder is nearly empty, and thus prevent the discharge of excessive amounts of odorous material.

If a compound of limited solubility is used as an odorizer, I have found that some of the more promising materials will evaporate too readily, and the concentration delivered decreased as the propane fuel is evaporated. I therefore propose, as a further example, to use with the fuel, a liquid of low volatility and limited miscibility, to dissolve a part of the odorous material to form a separate liquid phase which will deliver a sufficient concentration of the odorous material at all stages of emptying by evaporation. For this purpose, glycol can be used in a cylinder of propane fuel odorized by ammonia.

It has heretofore been proposed to add odorizing agents to a gas stream, but so far as I am aware, no proposal has been made prior to my invention to incorporate an odorizing agent directly into gas while the latter is in liquid condition and held under pressure in a cylinder or the like. The latter procedure presents problems which are not present in the odorizing of a gas stream. For instance, it is necessary to avoid the delivery of excessive concentration of a miscible odorizer from a near-empty cylinder, and it is necessary to control the concentration throughout delivery of a charge, when an odorizer of limited miscibility is used in connection with liquefied gas in a cylinder.

One prior inventor uses thio-acetone in a gas stream for odorizing purposes. He did not contemplate the use of organic sulfides in general, and dealt only with the odorizing of poisonous fuel gases, while I deal with non-poisonous gases which are stored in liquefied condition, and wish to introduce into the liquefied gas, only an amount of odorizer sufficient to odorize an explosive mixture (about 2.0% in air). A poisonous mixture of water or producer gas (0.05 to

0.10% in air) would require a much higher odor concentration.

From the foregoing it will be understood that my invention involves the following:

8 *First.*—The odorizing of liquefied petroleum gases to warn those present when there is a sufficient amount of such gas escaping to form an explosive mixture with air.

10 *Second.*—To impart the odorizing agent to the gas while the latter is in liquefied condition and held under pressure in a cylinder or the like.

12 *Third.*—To employ only such agents as will furnish an odor of the necessary strength during the entire delivery of the gas from the cylinder.

15 *Fourth.*—Avoiding the delivery of excessive concentration of a miscible odorizer from a near-empty cylinder by the introduction of a suitable retaining agent such as kerosene or glycol.

20 *Fifth.*—To provide a novel liquefied gas mixture.

It is believed that the invention may be readily understood from the foregoing description, but by way of reiteration it may be explained that at 25 the present time, large amounts of propane and the like are obtained from the treatment of natural gas, oil gas and the like. Such propane or its equivalent is placed under pressure and stored in gas-tight pressure cylinders, from 30 which the gas evaporates and is utilized by the consumer in gaseous condition. It is such liquefied petroleum gases as this which I propose to

odorize, and this I accomplish by the invention as explained above.

I am aware that substances other than those specifically mentioned are suitable for my purposes, and that changes may be made in the foregoing proposals, without departing from the spirit of the invention, as expressed in the claims.

What I claim and desire to secure by Letters Patent is:

1. A liquefied petroleum gas having admixed therewith a volatile odorizing agent in amount sufficient to odorize the leanest flammable mixture of said gas with air, and containing a substance having the characteristics of kerosene to avoid the delivery of excessive concentration of said odorizer from a substantially empty cylinder from which the gas is delivered.

2. Liquefied petroleum gas stored under pressure and having admixed therewith a miscible odorizing agent, and a substance having the characteristics of kerosene to prevent the delivery of excessive concentration of the odorizing agent from a substantially empty chamber from which the gas is delivered.

3. Liquefied petroleum gas containing a volatile odorizing agent and a substance dissolving the odorizing agent, but miscible to no more than a limited degree with the liquefied petroleum gas.

FREDERICK E. FREY.

35

11

40

11

45

11

50

11

55

11

60

11

65

11

70

11

75

11